

Patented Jan. 1, 1952

2,581,132

# UNITED STATES PATENT OFFICE

2,581,132

## LUBRICATING OIL

Roy F. Nelson, Alton J. Deutser, and Melvin R. Hefty, Port Arthur, Tex., assignors to The Texas Company, New York, N. Y., a corporation of Delaware

No Drawing. Application July 13, 1949,  
Serial No. 104,598

24 Claims. (Cl. 252—49.5)

1

This invention relates to a lubricating composition adapted to form a water-in-oil emulsion in the presence of water, and particularly to such a composition adapted to lubricate reciprocating steam engines of marine vessels and known as a marine engine oil.

For many years, marine engine oils have been compounded with about 10-20% or more by weight of blown rapeseed oil in mineral lubricating oil. The basic function of the blown rapeseed oil is generally considered to be as an emulsifier, although it imparts other properties to the lubricant composition which are both desirable and undesirable. Recently, due to a critical shortage of rapeseed oil as well as other equivalent fatty materials, with resultant increase in selling price and doubt concerning future availability, efforts have been made to develop the use of synthetic surface active materials, for the blown rapeseed oil. Since there is considerable water drip from the steam cylinders over the moving parts of marine engines, it is desirable that a lubricant of this type be capable of taking up a considerable amount of water. It is very important that this water be taken up in the form of a water-in-oil emulsion wherein the oil is in the continuous phase in order that the mixture will have good lubricating properties. In addition to this requirement of forming an emulsion of the proper water-in-oil type in the presence of water, the lubricant should also emulsify easily or readily under the mechanical mixing action of the moving parts of the engine such as the eccentrics, links, crosshead guides and slipper combs, and should also have satisfactory emulsion stability to resist separation of oil and water from the formed emulsion under the elevated temperature conditions encountered in the lubrication of the engine. Other properties desired include satisfactory adherence to the parts to be lubricated, satisfactory feeding of the lubricant through the customary wicks to the engine parts, proper viscosity of the lubricant per se and satisfactory emulsion consistency when the lubricant is emulsified with water.

One of the principal objects of the present invention is to provide a satisfactory lubricating composition of this character which forms a water-in-oil emulsion in the presence of water, and which is composed of at least about 90% by weight of mineral lubricating oil containing a small amount of available and highly effective emulsifier additive, or combination of emulsifier additives.

Another object of the present invention is to provide a marine engine oil of this type, which is highly satisfactory in service, and economical in manufacture and use, and which obviates the need for blown rapeseed oil in the composition.

Other objects and advantages of the present invention will be apparent from the following description and the appended claims.

The lubricating base of the present composi-

2

tion is a mineral lubricating oil of any known and available type, either from paraffin base or naphthalene base crudes, or from mixed base crudes. The viscosity of the mineral lubricating oil can vary throughout the lubricating oil viscosity range depending on the particular service conditions under which it is to be used, although for most marine engine oil service the viscosity at 100° F. (Saybolt Universal) may vary between about 400 and 1500 seconds. From the standpoint of providing a readily available and economical lubricating base, a naphthalene base lubricating oil which has been prepared by light acid treating, neutralizing, steaming and brightening, and which has a Saybolt Universal viscosity at 100° F. of about 500-1200 seconds, is preferred. As pointed out above, the mineral lubricating oil constitutes at least 90% by weight of the composition, preferably about 95% or more thereof.

In accordance with the present invention, this lubricating base is compounded with about 0.05-0.4% by weight based on the composition of a substituted glyoxalidine having the formula



30 where R is hydrogen or lower alkyl, R' is an alkyl or alkenyl group having from 10 to 30 carbon atoms, and X is a group selected from hydroxy-alkyl, amino-alkyl and amino-alkylene-imino-alkyl wherein the said alkyl radical of each group is lower alkyl. The preparation of compounds of this type by the reaction of a suitable soap-forming fatty acid with an alkylene polyamine is well known as described in Wilson Patent No. 2,267,965. Examples of suitable compounds of this type for purposes of the present invention are 1-amino ethyl 2-undecyl glyoxalidine; 1-amino ethyl 2-heptadecenyl glyoxalidine; 1-amino ethyl 2-heptadecyl glyoxalidine; 1-hydroxy ethyl 2-heptadecenyl glyoxalidine; 1-amino ethyl 2-heptadecenyl glyoxalidine; 1-amino ethyl ethyl-imino 2-heptadecenyl glyoxalidine; and 1-amino isopropyl 2-heptadecenyl 5-methyl glyoxalidine. A very satisfactory material of this character which is commercially available is 1-hydroxy ethyl 2-heptadecenyl glyoxalidine which is manufactured by Carbide and Carbon Chemicals Company under the name "Cationic Amine-220."

It has been discovered that, while a very large number of other known surface active agents tested were either incapable of forming a water-in-oil emulsion, as determined by the electrical conductivity of the emulsion, or required a high proportion in excess of 1-3% by weight to form a proper type of emulsion, the substituted glyoxalidines of the type described above were outstanding in possessing the property of forming a lubricating composition having the required

emulsion characteristics in the very low proportion range below 0.4% by weight. This is all the more unexpected since the prior art (cf. Wilkes 2,214,152) taught that these substituted glyoxalidines in a proportion above 0.5% by weight in a mineral lubricating oil produced a soluble oil type of composition capable of dispersing as an oil-in-water emulsion. In the following description, the compound 1-hydroxy ethyl 2-heptadecenyl glyoxalidine will be discussed by way of example as representative of the effective class of substituted glyoxalidines, any one of which can form the primary additive or emulsifier of the present composition.

While a satisfactory emulsifiable lubricant for certain purposes can be formed by compounding the substituted glyoxalidine in the small amount listed above in the mineral lubricating oil as the sole additive, it has been found that such composition can be further improved, particularly with respect to emulsion stability, by the addition of a second additive of a different type and which has a synergistic effect in the presence of the substituted glyoxalidine. Thus, in accordance with the present invention, there is also preferably incorporated in the composition about 0.1-1.0% by weight of a fatty acid partial ester of a hexahydric alcohol anhydride, wherein the fatty acid radical of said ester has from 10 to 30 carbon atoms. The various hexahydric alcohols, such as sorbitol, mannitol, dulcitol, and the like, are partially dehydrated and then esterified with soap-forming fatty acids, either saturated or unsaturated, to produce in well known manner compounds suitable for purposes of the present invention. The method of preparation of such compounds is described in Brown Patent No. 2,322,820. Specific examples of these compounds are sorbitan mono-oleate, sorbitan mono-laurate, manitan distearate and dulcitan trilaurate. A very satisfactory material of this type which is commercially available is sorbitan mono-oleate manufactured by Atlas Powder Company under the name "Span 80." In the following descrip-

4  
are suitable for purposes of the present invention.

In order to evaluate the effectiveness of the emulsifier additives with respect to emulsion formation and emulsion stability, the following Emulsion Test was employed as described in Federal Specification VV-L-791d Method 320.1.5. 40 milliliters of the mineral lubricating oil composition containing the additive or combination of additives were poured together with an equal quantity of water into a 100 ml. graduated cylinder. This cylinder was placed in a water bath maintained at 180° F. and allowed to stand until the contents reached the bath temperature. Then a copper plate stirring paddle (4 3/4" long, 3/4-1/8" wide and 1/8" thick) was lowered into the cylinder until its end was in position about 1/4" from the bottom of the cylinder. The mixed oil composition and water were then stirred by the paddle driven at 1500 R. P. M. by an electric motor for a 5-minute period, after which the paddle was removed. The graduate with the emulsified contents was kept in the bath for 60 minutes. The graduate was then removed and readings taken of the milliliters of oil separated, the milliliters of water separated and the milliliters of emulsion still present. This test was performed on each sample both with distilled water and with a 1% salt (NaCl) solution. In addition, each graduate following the 60-min. readings was allowed to stand for a further period of 16 hours at atmospheric temperature, and similar readings were again taken to indicate emulsion stability.

The following Table I sets forth the results obtained in this Emulsion Test, utilizing a naphthene base mineral lubricating oil having a Saybolt Universal viscosity at 100° F. of 515 seconds containing the specified amounts of additives A and B, where A is 1-hydroxy ethyl 2-heptadecenyl glyoxalidine and B is sorbitan mono-oleate. In the table, the three readings in each column for each sample under "Emulsion Test" signify from left to right the milliliters of oil separated, the milliliters of water separated and the milliliters of emulsion remaining.

TABLE I  
Naphthene base mineral lubricating oil—SUS at  
100° F. of 515

|    | Additive Conc.             |                            | Emulsion Test at 180° F. |         |                          |         |
|----|----------------------------|----------------------------|--------------------------|---------|--------------------------|---------|
|    | Per Cent<br>A <sup>1</sup> | Per Cent<br>B <sup>2</sup> | Distilled Water          |         | 1 Per Cent Salt Solution |         |
|    |                            |                            | 60 min.                  | 16 hrs. | 60 min.                  | 16 hrs. |
| 1  | 0.3                        | 1.0                        | T-0-80                   | 30-0-50 | T-0-80                   | 20-0-60 |
| 2  |                            | 1.0                        | 0-18-62                  | T-3-77  | T-0-80                   | 5-0-75  |
| 3  |                            | 3.0                        | T-0-80                   | T-0-70  | 8-0-72                   | 16-0-74 |
| 4  | 0.2                        | 0.1                        | T-0-80                   | 10-0-70 | T-0-80                   | 8-0-72  |
| 5  | 0.2                        | 0.3                        | T-0-80                   | 6-0-74  | T-0-80                   | 8-0-72  |
| 6  | 0.2                        | 0.5                        | T-0-80                   | 5-0-75  | 0-0-80                   | 8-0-72  |
| 7  | 0.3                        | 0.1                        | T-0-80                   | 20-0-60 |                          |         |
| 8  | 0.3                        | 0.3                        | T-0-80                   | 9-0-71  |                          |         |
| 9  | 0.3                        | 1.0                        | T-0-80                   | 7-0-73  |                          |         |
| 10 | 0.1                        | 0.3                        | T-0-80                   | 5-0-75  | 13-0-67                  | 20-0-60 |
| 11 | 0.1                        | 0.5                        | T-0-80                   | 4-0-76  | T-0-80                   | 4-0-76  |
| 12 | 0.1                        | 1.0                        | T-0-80                   | 5-0-75  | T-0-80                   | 4-0-76  |
| 13 | 0.15                       | 0.3                        | 1-0-79                   | 5-0-75  | T-0-80                   | 4-0-76  |
| 14 | 0.15                       | 0.5                        | T-0-80                   | 6-0-74  | T-0-80                   | 5-0-75  |
| 15 | 0.15                       | 1.0                        | T-0-80                   | 5-0-75  | T-0-80                   | 4-0-76  |
| 16 | (*)                        | (*)                        | T-0-80                   | 2-0-78  | 1-0-79                   | 2-0-78  |

T stands for trace.

<sup>1</sup> Additive A—1-hydroxy ethyl 2-heptadecenyl glyoxalidine.

<sup>2</sup> Additive B—Sorbitan mono-oleate.

<sup>3</sup> Conventional 20% blown rapeseed oil comp.

tion, sorbitan mono-oleate is listed by way of example as representative of these various partial esters of hexahydric alcohol anhydrides which

Sample 16 of the foregoing table was a conventional marine engine oil as previously employed, and consisted of a naphthene base lubri-

cating oil containing about 20% by weight of blown rapeseed oil. As shown, this conventional marine engine oil composition possessed good emulsion characteristics as illustrated by the 60-minute test with distilled water reported as "T-0-80," which signifies only a trace of oil separated, no water separated and 80 milliliters of emulsion still remaining. The similar test in the presence of the salt solution also indicates substantially complete emulsification, with only 1 ml. of oil separated, no water separated and 79 mls. of emulsion remaining. Likewise, the stability of the emulsion is good as shown by the results reported under the 16-hour columns.

Sample 1 of the table shows that the substituted glyoxalidine alone in a very low concentration effects substantially complete emulsification; however, the stability of the emulsion on standing is somewhat poorer with respect to oil separation. Samples 2 and 3 show that a high proportion of the order of about 3% by weight of the sorbitan mono-oleate is required to provide effective emulsification, although this material gives improved stability against oil separation. Samples 4-15 inclusive show that improved results with respect to both emulsion formation and emulsion stability are secured on an average basis by the combination of from 0.1 to 0.3% by weight of the glyoxalidine additive with 0.1 to 1.0% by weight of the sorbitan mono-oleate, although the results by this particular test for emulsion stability did not quite equal those of the conventional blown rapeseed oil composition. However, a lubricant composition consisting of the lubricating base with the listed proportions of these two additives constitutes a satisfactory emulsifiable lubricating material for certain purposes, and the total additive concentration is much less than in the conventional blown rapeseed composition.

In addition to forming a tight emulsion of the water-in-oil type which is stable against separation on standing, it is desirable that the composition easily and rapidly form such an emulsion under conditions encountered in marine engine lubrication. A test for evaluating this characteristic will now be described. The apparatus em-

ployed was the same as that described above in connection with the Emulsion Test at 180° F. However, in this case the mixture of 40 ml. of distilled water and 40 ml. of the composition under test were maintained at a temperature of 75° F., and intermittent stirring periods of 30 seconds on and 60 seconds off were employed. This intermittent stirring was continued until complete emulsification had been attained, that is, when the mixture changed from a thin curdy non-homogeneous appearance of tan color to a cream-colored viscous smooth and homogeneous appearing emulsion. The number of stirring periods required to attain that result was reported under the test heading of Ease of Emulsification.

In order to further improve the emulsion characteristics of the composition, particularly from the standpoint of ease of emulsification, there may be added to the composition in accordance with the present invention about 0.05-0.5% by weight of a linear isoolefinic polymer having a molecular weight in excess of 2,000 and preferably in excess of 5,000. The manufacture of high molecular weight polymers of this type, such as from isobutylene, is well known as described in Otto et al. Patent No. 2,084,501. These high molecular weight polymers are formed by condensation at low temperatures in the presence of a suitable catalyst such as  $BF_3$ ; and the higher molecular weight extremely viscous or solid products having a molecular weight from 10,000 to 20,000 or higher are conveniently employed as a mineral lubricating oil solution or concentrate of the polymer. A very satisfactory material of this type for purposes of the present invention is the viscous stringy lubricating oil concentrate containing about 50% by weight of an isobutylene polymer having a molecular weight of around 20,000 which is manufactured by the Enjay Company under the name "Paramac." In addition to improving the emulsion characteristics of the composition, this polymer additive also improves the adherence of the composition to the parts being lubricated.

The following Table II sets forth the results obtained on various compositions in the Emul-

TABLE II

|  | Additive Conc. Per Cent |   |                | Emulsion Test at 180° F. |                      | Ease of Emulsification—Stirring Periods |
|--|-------------------------|---|----------------|--------------------------|----------------------|-----------------------------------------|
|  | A                       | B | C <sup>1</sup> | Distilled Water          | 1 Per Cent Salt Sol. |                                         |

BASE OIL—NAPHTHENE BASE LUBRICATING OIL—S. U. S. AT 100° F. OF 1123

|    |     |                  |     |            |           |    |
|----|-----|------------------|-----|------------|-----------|----|
| 1  |     |                  | 0.5 | 40-36-4-5  |           |    |
| 2  |     |                  | 0.1 | 40-40-0-5  |           |    |
| 3  |     |                  | 0.5 | T-19-31-60 |           |    |
| 4  |     |                  | 0.3 | 1-20-59-60 |           |    |
| 5  |     |                  | 0.1 | 1-18-61-60 |           |    |
| 6  | 0.3 |                  | 0.5 | T-0-80-60  |           |    |
| 7  | 0.3 |                  | 0.3 | T-0-80-60  |           |    |
| 8  | 0.2 | 0.3 <sup>2</sup> | 0.5 | T-0-80-60  | T-0-80-60 | 4  |
| 9  | 0.2 | 0.3              | 0.3 | T-0-80-60  | T-0-80-60 | 6  |
| 10 | 0.2 | 0.3              | 0.1 |            | T-0-80-60 |    |
| 11 | 0.2 | 0.3              | 0.2 |            |           | 10 |

BASE OIL—NAPHTHENE BASE LUBRICATING OIL—S. U. S. AT 100° F. OF 769

|    |     |     |     |           |           |     |
|----|-----|-----|-----|-----------|-----------|-----|
| 12 | 0.2 | 0.3 | 0.4 | T-0-80-60 | T-0-80-60 | 5   |
| 13 | 0.2 | 0.3 | 0.4 | T-0-80-60 | T-0-80-60 | 9   |
| 14 | 0.2 | 0.3 | 0.2 | T-0-80-60 | T-0-80-60 |     |
| 15 | 0.2 | 0.3 | (?) |           |           | 10+ |
| 16 | (?) | (?) | (?) |           |           | 10+ |

<sup>1</sup> Additive C—Lubricating oil concentrate of about 50% by weight of isobutylene polymer of m. w. about 20,000.

<sup>2</sup> Conventional 20% blown rapeseed oil comp.

sion Test at 180° F. as well as the Ease of Emulsification Test, wherein additives A and B are respectively the same as in Table I and additive C is a lubricating oil concentrate containing about 50% by weight of isobutylene polymer of molecular weight around 20,000. In this table, the results under Emulsion Test are reported in four numbers, which signify from left to right the ml. of oil separated, the ml. of water separated, the ml. of emulsion remaining, and the time in minutes after stirring was stopped that the readings were taken.

As will be noted from samples 1 and 2 of the foregoing table, the polymer additive alone is lacking in emulsion forming characteristics, under these conditions as evidenced by almost complete separation into oil and water phases just five minutes after stirring was terminated. Samples 3-5 show that the combination of the polymer additive with the partial ester of the hexahydric alcohol anhydride is also comparatively ineffective, since there is substantial water separation at the termination of the 60-minute test. On the other hand, the combination of the polymer additive with the glyoxalidine primary additive provides highly effective emulsification, as illustrated by samples 6 and 7, and constitutes a very satisfactory composition for certain purposes. Samples 8-14 inclusive show that the combination of the three additives provides the superior emulsification characteristics which are necessary in a marine engine lubricant; and, in comparison with sample 15 wherein the polymer additive was omitted, show that the ease of emulsification is materially improved by the presence of the third polymer additive, as illustrated by the number of stirring periods in the Ease of Emulsification Test. In fact, the composition containing the three additives in the proportions set forth shows improved ease of emulsification under the conditions of this test over the conventional blown rapeseed oil composition.

From the foregoing tables, it will be noted that satisfactory compositions prepared in accordance with the present invention contain extremely low proportions of additive in comparison to the conventional blown rapeseed oil composition of 10-20% additive content. Consequently, in order to produce a lubricating composition of similar grade or viscosity in accordance with the present invention, it is necessary to employ a heavier base oil. It has been found that, while the lubricating composition per se of the present invention employing the heavier base oil with the smaller proportion of additives may have a comparable viscosity to the conventional blown rapeseed oil product, nevertheless when the two are emulsified with water the resulting emulsions are materially different in fluidity. Thus the present composition when formed into a 1:1 emulsion with water possesses a thicker consistency as measured by a Brookfield viscosimeter at 100° F. than a 1:1 water emulsion of the conventional blown rapeseed oil composition of comparable initial viscosity. It has been further found that the addition of about 0.1-0.5% by weight of refined wool grease or lanolin to the foregoing compositions of the present invention reduces the emulsion consistency thereof to values more in line with the emulsion viscosities of the conventional rapeseed oil product. This is illustrated in the following Table III, where additives A, B and C

are the same as in Tables I and II and additive D is lanolin.

TABLE III  
Naphthalene base oil (S. U. S. at 100° F. of 769)

|    | Additive Conc. |     |     |                | Viscosity of 1-1 Emulsion Centipoises at 100° F. | Emulsion Test at 180° F. |
|----|----------------|-----|-----|----------------|--------------------------------------------------|--------------------------|
|    | A              | B   | C   | D <sup>1</sup> |                                                  |                          |
| 10 | 0.2            | 0.3 | 0.4 | —              | 3,680                                            | 0-0-80-60                |
| 1  | 0.2            | 0.3 | 0.2 | 0.1            | 2,320                                            | 0-0-80-60                |
| 2  | 0.2            | 0.3 | 0.2 | 0.5            | 2,320                                            | 1-0-79-60                |
| 3  | 0.2            | 0.3 | 0.2 | 0.2            | —                                                | 0-0-80-60                |
| 4  | 0.2            | 0.3 | 0.2 | 0.2            | —                                                | 1-0-79-60                |
| 5  | 0.2            | 0.2 | 0.2 | 0.2            | 2,240                                            | 1-0-79-60                |
| 6  | (2)            | (2) | (2) | (2)            | 1,600                                            | 0-0-80-60                |

<sup>1</sup> Additive D—Lanolin.

<sup>2</sup> Conventional 20% blown rapeseed oil comp.

As shown by sample 1 in comparison with sample 6 of the foregoing table, the emulsion viscosity of the present composition in the absence of added lanolin is materially higher than that of the conventional rapeseed oil composition of comparable non-emulsified viscosity. Samples 2-5 inclusive show the effect of the added lanolin in the present composition with respect to reduction in emulsion consistency. It is to be noted that the addition of the lanolin to the present composition does not detract from the emulsion characteristics thereof as shown by the Emulsion Test at 180° F. In addition to the emulsion viscosity thinning effect, the lanolin also adds cileness and a smoothing effect to the oil composition and to the water emulsion formed therefrom.

Very satisfactory compositions for purposes of the present invention are represented by samples 2, 3 and 5 of Table III although products represented by samples 1 and 4 are well suited to other uses. Complete tests on samples 4 and 5 are set forth by way of example in the following Table IV:

TABLE IV  
Tests on Compositions 4 and 5 of Table III

|    | Tests                                            | Comp. 4    | Comp. 5   |
|----|--------------------------------------------------|------------|-----------|
| 45 | Gravity °API                                     | 21.2       | 21.2      |
|    | Flash, O. Cleve., °F.                            | 410        | 400       |
|    | Fire, Cleve., °F.                                | 455        | 470       |
|    | Visc., S. U. at 100° F.                          | 802        | 797       |
|    | Visc., S. U. at 130° F.                          | 293        | 299       |
|    | Visc., S. U. at 210° F.                          | 64         | 64        |
|    | Viscosity Index                                  | 30.8       | 31.7      |
|    | Color, $\frac{1}{2}$ " Love. Cell                | 115        | 110       |
|    | Pour, °F.                                        | -15        | -15       |
|    | Corr., Cu Strip, 1 hr. at 212° F.                | Neg.       | Neg.      |
|    | Ash, Per Cent.                                   | 0.007      | 0.005     |
|    | Emulsion Test at 180° F.:                        |            |           |
| 55 | Distilled Water                                  | 0-0-80-60  | 1-0-79-60 |
|    | 1% Salt Solution                                 | 10-0-70-60 | 1-0-79-60 |
|    | Ease of Emulsification:                          |            |           |
|    | Stirring Periods at 75° F.                       | 3          | 3         |
|    | Emulsion Stability—16 hours at room temperature: |            |           |
|    | Distilled Water                                  | 5-0-75     | 4-0-76    |
| 60 | 1% Salt Solution                                 | 28-0-52    | 9-0-71    |

The foregoing table again illustrates the synergistic effect of the sorbitan mono-oleate in combination with other additives in repressing oil separation from the emulsion. This is shown by the Emulsion Test at 180° F. in the presence of 1% salt solution, and also by the Emulsion Stability Test. It is to be noted that both compositions show excellent results by the above described Ease of Emulsification test.

While composition 5 of Tables III and IV provided excellent lubrication in full scale marine engine tests, it did not emulsify as readily in the eccentric pans as conventional 20% blown rapeseed compositions, although the emulsion char-

acteristics were entirely satisfactory on the smaller bearing surfaces on other parts of the engine such as links and connecting rods. A new test was therefore developed duplicating in miniature the motion of the engine eccentrics encountered on ships. For this purpose, a motor driven horizontal shaft equipped with a 4" diameter eccentric (eccentricity of 1 in.) was maintained with the eccentric dipping within a semi-circular pan (3½" radius x 2½" wide) so that the eccentric at the extreme limit of its movement was about ½" from the semi-circular side of the pan. 250 milliliters of water and 250 milliliters of the oil composition under test were added to the pan, thereby bringing the level of the oil-water mixture to about 1" below the shaft axis. With this oil-water mixture maintained at 95-100° F., the shaft and eccentric were rotated at 125/R. P. M.; and the time in minutes for effecting complete emulsification of the mixture as determined visually in the manner described above was recorded. This test termed the Eccentric Emulsification Test was found to correlate well with actual service.

To further improve the ease of emulsification of the lubricant compositions of the present invention, as determined by the Eccentric Emulsification Test, the addition of about 0.05-0.4% by weight of a saturated fatty acid ester of an alkyloamine, where the saturated fatty acid contains 10 to 30 carbon atoms in the molecule, is made in accordance with the present invention. Any one of the mono-, di-, and tri-alkyloamines, wherein the alkyloamine is combined with a soap-forming saturated fatty acid, can be employed. Other types of carboxylic acids, such as naphthenic acids and unsaturated fatty acids, are excluded. Examples of suitable materials of this type include triethanolamine stearate, diethanolamine palmitate, tripropanolamine behenate, diethyl ethanolamine stearate and triethanolamine myristate. A preferred material for this purpose from the standpoint of availability is triethanolamine stearate, and this is listed in the following tables by way of illustration.

Table V illustrates the results obtained in the above-described Eccentric Emulsification Test on compositions prepared in accordance with the present invention in comparison with the conventional rapeseed oil product.

TABLE V

|      | Composition                                                                 | Eccentric Emulsification Test Time in min. |
|------|-----------------------------------------------------------------------------|--------------------------------------------|
| 1... | Conventional 20% blown rapeseed oil comp.                                   | 18, 14, 11.                                |
| 2... | Comp. 5 of Table III                                                        | 60, 65.                                    |
| 3... | Comp. 5 with equal amt. of additive A replaced with 0.1% TEAS. <sup>1</sup> | 14.                                        |
| 4... | Comp. 5 with equal amt. of additive A replaced with 0.15% TEAS.             | 10.                                        |
| 5... | Comp. 5+0.3% TEAS.                                                          | 7.                                         |
| 6... | Comp. 5+0.2% TEAS.                                                          | 9.                                         |
| 7... | Comp. 5+0.1% TEAS.                                                          | 14.                                        |
| 8... | Comp. 5+0.05% TEAS                                                          | 45+.                                       |

<sup>1</sup> Triethanolamine stearate.

Samples 1 and 2 of the foregoing table show that the preferred composition 5 of Tables III and IV requires approximately 4-5 times as long to com-

pletely emulsify in the Eccentric Emulsification Test as does the conventional rapeseed oil composition. On the other hand, samples 3-8 inclusive show that the presence of the small proportion of added triethanolamine stearate, either as a partial replacement for the glyoxalidine additive or as a further additive to the composition, materially reduces the emulsification time by this test and renders the product at least equal if not superior to the conventional blown rapeseed oil composition with respect to ease of emulsification. While the saturated fatty acid esters of the alkyloamines have been found effective for this purpose, the unsaturated fatty acid esters and the naphthenic acid esters are substantially ineffective. For example, the addition of from 0.1 to 0.2% triethanolamine oleate and from 0.1 to 0.2% triethanolamine naphthenate to the said composition 5 (also containing 1% sulfurized lard oil) gave times of 71-90 min. and 90 min. respectively in the said Eccentric Emulsification Test. A proportion of around 0.1-0.2% of triethanolamine stearate in the composition is preferred for optimum overall results, since this material is not very soluble in mineral oil and higher proportions may result in some gel formation in the composition on storage at low temperatures of the order of 25-35° F.

Finally, in accordance with the present invention, the film strength and extreme pressure properties of the foregoing compositions may be improved by the addition of a sulfurized vegetable or animal oil wherein the sulfur is in a combined non-corrosive form so as to give a negative or non-corrosive result in the Copper Strip Corrosion Test at 100° F. Any of the various animal and vegetable oils which are sulfurized at elevated temperatures and then blown with steam to remove H<sub>2</sub>S and render them non-corrosive, can be employed for this purpose, since these materials are found compatible with the other additives and do not interfere with or detract from the emulsifying properties of the composition. Examples of suitable sulfurized oils of this type for the present purpose are sulfurized lard oil, sulfurized rapeseed oil, sulfurized sperm oil, sulfurized cottonseed oil, and sulfurized palm oil. The sulfurized oil should be employed in the composition in a portion range of about 0.3-3.0% by weight and preferably about 0.5-1.5%.

A very satisfactory additive of this type which is prepared from a readily available material is sulfurized lard oil which was manufactured as follows: 90% by weight of No. 1 lard oil was mixed with 10% by weight of powdered sulfur and the mixture raised to a temperature of 400° F. in eight hours with continuous stirring. The mixture was then held at this temperature for an additional three hours with intermittent stirring, and then blown with live steam for at least two hours to remove H<sub>2</sub>S. The product was allowed to cool to 250° F. with stirring and then drawn through a filter. The resulting sulfurized lard oil contains from about 6 to 10% of combined sulfur, generally around 7.5%, and is negative in the Copper Dish Corrosion Test at 100° F. A desirable characteristic of these sulfurized oils containing combined sulfur is that, while they are non-corrosive at lower temperatures, they have the ability to release sulfur at exceptionally high temperature which may be occasionally encountered in service. The sulfurized

## 11

lard oil per se gives a positive test in the Copper Strip Corrosion Test at 212° F. However, the lubricating composition of the present invention contains such a small proportion of the sulfurized oil that the composition passes the Copper Strip Corrosion Test at 212° F.

Results obtained on a typical composition of the present invention with the addition of typical sulfurized oils, demonstrating the improvement in extreme pressure properties, are set forth in the following Table VI. The tests employed include the standard SAE and Timken extreme pressure tests for lubricants which are well known. In addition, the table gives the results of a so-called modified Southern Pacific Bearing Temperature Rise Test, which consists of gradually loading a brass bearing on a rotating bushing until the bearing temperature reaches 250° F. The pressure on the bearing in pounds per sq. inch which is required to raise the bearing temperature to 250° F. is reported. Inasmuch as the Timken and SAE tests encounter extremely high skin temperatures far above those encountered in marine lubrication, the Southern Pacific test is thought to give a more practical measure of the performance of marine lubricants.

TABLE VI

|   | Composition                         | SAE Test 500<br>r. p. m. | Timken Test<br>O. K. Score | Mod. SP Bearing<br>Temp. Rise Test<br>lb./in. <sup>2</sup> for 250° F.<br>Temp. |
|---|-------------------------------------|--------------------------|----------------------------|---------------------------------------------------------------------------------|
| 1 | Conv. 20% blown rapeseed oil        | 85-110-95                | 15 20                      | 1200 1200                                                                       |
| 2 | Comp. 5 of Table III                | 110-100-70               | 7 9                        | 700 700                                                                         |
| 3 | Comp. 5, 1% sulfurized lard oil     | 77-104-75                | 15 20                      | 1200 1200                                                                       |
| 4 | Comp. 5, 1% sulfurized rapeseed oil | 82-110-84                | 10 15                      |                                                                                 |
| 5 | Comp. 5, 1% sulfurized sperm oil    | 128-106-128              | 10 15                      |                                                                                 |

As will be noted from the foregoing table, the SAE test rated the various compositions essentially the same within the accuracy of the test procedure. However, the Timken and Southern Pacific tests show the conventional blown rapeseed oil composition to have better extreme pressure properties than composition 5 of Table III. Sample 3 of this table shows that when 1% of sulfurized lard oil prepared as described above was added to said composition 5, the extreme pressure properties of the resulting lubricant were essentially equal to the conventional blown rapeseed oil composition by these various tests.

The following Table VII shows the results obtained in the Eccentric Emulsification Test on the preferred composition 5 of Table III when triethanolamine stearate, and both the latter and sulfurized lard oil, are added.

TABLE VII

|   | Composition                    | Eccentric Emul-<br>sification Test<br>Time in Min. |
|---|--------------------------------|----------------------------------------------------|
| 1 | Comp. 5 of Table III+0.2% TEAS | 9                                                  |
| 2 | (1)+1% sulfurized lard oil     | 8                                                  |
| 3 | Comp. 5+0.1% TEAS              | 14                                                 |
| 4 | (3)+1% sulfurized lard oil     | 12                                                 |

As indicated by this table, the ease of emulsification of the composition is not affected adversely by the addition of the sulfurized lard oil, and in fact appears to be somewhat improved.

The specific compositions described above are given by way of example and the present invention includes compositions composed of the base oil plus the specified proportions of the glyoxali-

## 12

dine additive with other combinations of the foregoing described supplementary additives. For example the glyoxalidine additive may be used in combination with only the alkylolamine ester additive, where the emphasis is on ease of emulsification by the Eccentric Emulsification Test as opposed to stability of the emulsion. The invention also includes the foregoing composition containing as a third additive either the partial hexitol anhydride ester to provide improved stability against oil separation, or the iso-olefinic polymer to provide improved adherence and still better all-around emulsion characteristics. A preferred composition for purposes of the present invention and possessing excellent overall emulsion characteristics is the following:

|                                                                                        | Per cent<br>by weight |
|----------------------------------------------------------------------------------------|-----------------------|
| Mineral lubricating oil                                                                | 94.2-99.75            |
| 1-hydroxy alkyl 2-C <sub>10</sub> to C <sub>30</sub> alkenyl glyoxalidine              | 0.05-0.4              |
| Alkylolamine C <sub>16</sub> -C <sub>30</sub> saturated fatty acid ester               | 0.05-0.4              |
| Hexahydric alcohol anhydride C <sub>10</sub> -C <sub>30</sub> fatty acid partial ester | 0.1-1.0               |
| Linear iso-olefinic polymer having molecular weight over 5,000                         | 0.05-0.5              |

To further improve the composition as listed immediately above with respect to emulsion consistency, and to improve the oiliness of both the oil and the emulsion, about 0.1 to 0.5% by weight of lanolin can be added. In addition, to provide extreme pressure properties and suppress gel formation, about 0.3-3.0% by weight of a non-corrosive sulfurized fatty oil extreme pressure agent can be added.

To further illustrate the present invention, the following example is given of a composition which has functioned very satisfactorily in actual service as a marine engine oil. The following Table VIII sets forth the weight and proportions of ingredients employed to produce a typical batch of this marine engine oil, together with tests on the individual ingredients employed in producing the batch.

TABLE VIII

| Ingredients                                                               | Wt. in lbs. | Wt. per cent |
|---------------------------------------------------------------------------|-------------|--------------|
| Naphthalene base mineral lubricating oil                                  | 22,732      | 98.0         |
| 1-hydroxyethyl 2-heptadecenyl glyoxalidine                                | 46.4        | 0.2          |
| Sorbitan mono-oleate                                                      | 46.4        | 0.2          |
| Refined wool grease                                                       | 46.4        | 0.2          |
| 50% lubricating oil concentrate of isobutylene polymer of m. w. of 20,000 | 46.4        | 0.2          |
| Triethanolamine stearate                                                  | 46.4        | 0.2          |
| Sulfurized lard oil                                                       | 232         | 1.0          |
| Total                                                                     | 23,196      | 100.0        |

## Tests on ingredients

|                                                                                                                                  | Tests on material used in batch     |
|----------------------------------------------------------------------------------------------------------------------------------|-------------------------------------|
| Naphthalene base lubricating oil:                                                                                                |                                     |
| Gravity, °API                                                                                                                    | 21.2                                |
| Flash -O-Clev., °F.                                                                                                              | 415                                 |
| Fire, Cleve., °F.                                                                                                                |                                     |
| Visc., S. U. at 100° F.                                                                                                          | 759                                 |
| Visc., S. U. at 210° F.                                                                                                          | 62.8                                |
| Color, Lovi. 1/2" cell                                                                                                           | 120                                 |
| Pour, °F.                                                                                                                        | -10                                 |
| Neut. No.                                                                                                                        |                                     |
| Ash, per cent                                                                                                                    | 0.005                               |
| Corr., Cu. Strip, 3 hrs. at 212° F.                                                                                              |                                     |
| 1-hydroxyethyl 2-heptadecenyl glyoxalidine:                                                                                      |                                     |
| Gravity, 20° C./20° C.                                                                                                           | 0.9375                              |
| Visc., S. U. at 100° F.                                                                                                          | 800                                 |
| Visc., c. p. at 100° F.                                                                                                          | 159                                 |
| Color, ASTM                                                                                                                      | 4.0                                 |
| Emulsion test at 180° F., 0.2% solution in naphthalene base lubricating oil (S. U. at 100° F. of about 300) with distilled water | 1-0-79-60                           |
| Sorbitan mono-oleate:                                                                                                            |                                     |
| Sap. No.                                                                                                                         | 150                                 |
| Hydroxyl No.                                                                                                                     | 221                                 |
| Acid No.                                                                                                                         | 5.9                                 |
| Visc., c. p. at 25° C.                                                                                                           | 1100                                |
| Sp. Gr.                                                                                                                          | 0.9923                              |
| Refined wool grease:                                                                                                             |                                     |
| Color, NPA, 90% diluted with water white kerosine                                                                                | 1.5                                 |
| Melting point, °F.                                                                                                               |                                     |
| Free fatty acid (as oleic), per cent                                                                                             | 0.14                                |
| Sap. No.                                                                                                                         | 94                                  |
| Iodine No.                                                                                                                       |                                     |
| Water, per cent                                                                                                                  | 0.2                                 |
| Ash, per cent                                                                                                                    | 0.05                                |
| Lube oil conc. of isobutylene polymer:                                                                                           |                                     |
| Appearance                                                                                                                       | Viscous stringy pale colored liquid |
| Triethanolamine stearate:                                                                                                        |                                     |
| Color, FAC                                                                                                                       | 1                                   |
| Melting point, °C.                                                                                                               | 41.8                                |
| pH of 5% aqueous sol. at 25° C.                                                                                                  | 8.7                                 |
| Gravity at 25/25° C.                                                                                                             | 1.0229                              |
| Sulfurized lard oil:                                                                                                             |                                     |
| Gravity, °API                                                                                                                    | 13.9                                |
| Visc., S. U. at 210° F.                                                                                                          | 245                                 |
| Sulfur, per cent                                                                                                                 | 7.66                                |

Manufacture of any of the compositions previously described may be carried out by simple mixing of the ingredients in any suitable vessel at moderately warm temperatures. In the preparation of the foregoing batch, the mineral lubricating oil was charged to a steam heated kettle equipped with a mechanical stirrer. A small side mixer separate from the blending kettle was preferably provided for incorporating the additives, with connections permitting the oil to be pumped from the large kettle up through the bottom of the side mixer, and permitting oil overflow from the side mixer to run back into the large kettle. This side mixer is particularly advantageous when a normally solid material of the character of the alkylolamine fatty acid ester is included in the batch.

After charging the oil to the large kettle, stirring was started and steam heat was turned on to raise the kettle and contents to a temperature of about 120-130° F. which was thereafter maintained in the manufacture of the batch. The side mixer was then started, utilizing a pumping rate of about 50 gallons or more per minute from the large kettle through the recirculating line to the side mixer and back to the kettle. The indicated amounts of the substituted glyoxalidine, the sorbitan mono-oleate, the refined wool grease and the isobutylene polymer concentrate were then added in order to the side kettle, with about 5-10 minutes being allowed for recirculation between the addition of each material.

At this point recirculation through the side mixer, which was full of the composition, was discontinued. The contents of the side mixer were then heated to 180° F. with stirring. The indicated amount of triethanolamine stearate was added to the side mixer. Heating was continued to a temperature of about 210-220° F. and this temperature was maintained for about 15 minutes to insure complete solution of the additive. Recirculation was then resumed. The concentrate was transferred to the main portion of the composition in the large kettle which meanwhile had been maintained at 120-130° F. The indicated amount of sulfurized lard oil was then added directly to the large kettle and stirring was continued for about 1/2 hour until the finished product was bright and clear. The final composition was then drawn to tankage.

Typical tests obtained on the foregoing composition, together with test specifications for the product are set forth in the following Table IX:

TABLE IX

|    | Tests on Batch                                                                                                                                                                                                                        | Specifications                                                                                                                      |
|----|---------------------------------------------------------------------------------------------------------------------------------------------------------------------------------------------------------------------------------------|-------------------------------------------------------------------------------------------------------------------------------------|
| 40 |                                                                                                                                                                                                                                       |                                                                                                                                     |
| 45 | Gravity ° API<br>Flash, O-Clev., ° F.<br>Visc., S. U. at 100° F.<br>Visc., S. U. at 130° F.<br>Visc., S. U. at 210° F.<br>Viscosity Index<br>Color, 1/2" Lovi. Cell<br>Pour, ° F.<br>Corr., Cu. Strip, 3 hrs. at 212° F.<br>Neut. No. | 20.9<br>410<br>774<br>296<br>65.1<br>43.1<br>170<br>-25<br>Neg.<br>0.50                                                             |
| 50 | Sap. No.<br>Wick Feed Test<br>Emulsion Test VV-L-79d Method<br>320.1.5.<br>Eccentric Emulsification Test<br>Emulsion Stability—Oil separation after 2 hrs. at 180° F. in ml.                                                          | 2.8<br>Passes<br>0-0-80-60<br>8, 11, 9, 10<br>0                                                                                     |
| 55 |                                                                                                                                                                                                                                       | 18.0-22.0.<br>375 min.<br>280-310.<br>62.5-66.5.<br>150-200.<br>10 max.<br>Neg.<br>30% retain flow in 14 days.<br>30 max.<br>1 max. |

The Wick Feed Test of the foregoing table is U. S. Government Method 200.1, and is designed to indicate the manner in which the oil composition will feed through the wicks in marine engine service. This test employs a brass oil container of about 1 quart capacity fitted in the center with a brass tube of 1/2" internal diameter serving as an oil-way and feeding into a graduated cylinder. A wick is employed which is composed of eight strands of worsted zephyr of the best quality, pure, long-fiber, cream white fine wool, thoroughly washed, scoured and carded, but not dyed or subjected to any chemical process. The strands are 4-ply soft spun and twisted; and the separate plies are of uniform thickness throughout their entire length. A wick support in the form of a hook of copper wire is employed which grips the outlet end of the wick below the level

of the oil. The wick is dipped in the oil and placed in a position with the oil container filled so that the lift of the wick is  $\frac{1}{4}$ "; and this lift is maintained at from  $\frac{1}{4}$  to  $\frac{1}{2}$ " during the test. The flow of oil into the graduated cylinder is measured at the end of 24 and 48 hours and again at the end of 14 days. The Government specification requires that the flow at the end of 14 days shall be at least 30% of the flow during the initial periods of the test.

The foregoing Table IX also includes an Emulsion Stability Test which is more severe than the room temperature test previously described and is employed in conjunction with the Eccentric Emulsification Test. After completion of the Eccentric Emulsification Test, 100 mls. of the emulsified mixture from the pan are transferred to a graduate and the latter is placed in a bath maintained at  $180^{\circ}$  F. After two hours in the bath, the number of mls. of separated oil and/or water are recorded.

While the invention has been described above particularly as a marine engine oil, it is to be understood that the invention is not limited to that service but is applicable to any lubricating service where water may be encountered and it is desired that a water-in-oil emulsion shall be produced in a manner to effectively remove the water from contact with the metal parts and to maintain the latter coated with an adherent lubricating film.

Obviously many modifications and variations of the invention, as hereinbefore set forth, may be made without departing from the spirit and scope thereof and, therefore, only such limitations should be imposed as are indicated in the appended claims.

We claim:

1. A lubricating composition adapted to form a water-in-oil emulsion in the presence of water, with the water in the discontinuous phase, comprising a mineral lubricating oil as the predominant constituent, and constituting at least 90% by weight of the composition, and about 0.05-0.4% by weight based on the composition of a substituted glyoxalidine having the formula



where R is selected from the group consisting of hydrogen and lower alkyl, R' is selected from the group consisting of alkyl and alkenyl radicals having from 10 to 30 carbon atoms, and X is selected from the group consisting of hydroxy-lower alkyl, amino-lower alkyl and amino-alkylene-imino-lower alkyl.

2. A lubricating composition according to claim 1, wherein R' is an alkenyl group having 15 to 20 carbon atoms, and X is a hydroxy alkyl group.

3. A lubricating composition according to claim 2, wherein the substituted glyoxalidine is 1-hydroxyethyl 2-heptadecenyl glyoxalidine.

4. A lubricating composition adapted to form a water-in-oil emulsion in the presence of water, with the water in the discontinuous phase, comprising a mineral lubricating oil as the predominant constituent, and constituting at least 90% by weight of the composition, about 0.05-0.4%

by weight on the basis of the composition of a substituted glyoxalidine having the formula



10 where R is selected from the group consisting of hydrogen and lower alkyl, R' is selected from the group consisting of alkyl and alkenyl radicals having from 10 to 30 carbon atoms, and X is selected from the group consisting of hydroxy-lower alkyl, amino-lower alkyl and amino-alkylene-imino-lower alkyl, and about 0.1-1.0% by weight based on the composition of a higher fatty acid partial ester of a hexahydric alcohol anhydride, the fatty acid radical of said ester having from 10 to 30 carbon atoms.

15 5. A lubricating composition according to claim 4, wherein said ester is sorbitan mono-oleate.

6. A lubricating composition according to claim 5, wherein said glyoxalidine compound is 1-hydroxyethyl 2-heptadecenyl glyoxalidine.

20 7. A lubricating composition adapted to form a water-in-oil emulsion in the presence of water, with the water in the discontinuous phase, comprising a mineral lubricating oil as the predominant constituent, and constituting at least 90% by weight of the composition, about 0.05-0.4% by weight on the basis of the composition of a substituted glyoxalidine having the formula



30 35 where R is selected from the group consisting of hydrogen and lower alkyl, R' is selected from the group consisting of alkyl and alkenyl radicals having from 10 to 30 carbon atoms, and X is selected from the group consisting of hydroxy-lower alkyl, amino-lower alkyl and amino-alkylene-imino-lower alkyl, and about 0.05-0.4% by weight based on the composition of a saturated higher fatty acid ester of an alkylolamine where the saturated fatty acid contains 16 to 30 carbon atoms.

40 50 60 7. A lubricating composition according to claim 7, wherein the ester is a stearic acid ester.

8. A lubricating composition according to claim 8, wherein the ester is triethanolamine stearate.

55 9. A lubricating composition according to claim 7, wherein the composition also contains about 0.1-1.0% by weight based on the composition of a higher fatty acid partial ester of a hexahydric alcohol anhydride, the fatty acid radical of said ester having from 10 to 30 carbon atoms.

10. A lubricating composition according to claim 10, wherein the partial ester is sorbitan mono-oleate.

65 11. A lubricating composition according to claim 7, wherein the composition also contains about 0.3-3.0% by weight based on the composition of a non-corrosive sulfurized fatty oil extreme pressure agent which is compatible with the said substituted glyoxalidine and the said ester and does not detract from the emulsification properties thereof.

12. A lubricating composition according to claim 12, wherein the said sulfurized fatty oil

is sulfurized lard oil containing about 5-15% of combined sulfur.

14. A lubricating composition adapted to form a water-in-oil emulsion in the presence of water, with the water in the discontinuous phase, comprising a mineral lubricating oil as the predominant constituent and constituting at least 90% by weight of the composition, about 0.05-0.4% by weight on the basis of the composition of a substituted glyoxalidine having the formula



where R is selected from the group consisting of hydrogen and lower alkyl, R' is selected from the group consisting of alkyl and alkenyl radicals having from 10 to 30 carbon atoms, and X is selected from the group consisting of hydroxy-lower alkyl, amino-lower alkyl and amino-alkylene-imino-lower alkyl, and about 0.05-0.5% by weight based on the composition of a linear iso-olefinic polymer having a molecular weight in excess of 2,000.

15. A lubricating composition according to claim 14, said composition also containing about 0.05-0.4% by weight based on the composition of a saturated fatty acid ester of an alkylolamine where the saturated fatty acid contains 10 to 30 carbon atoms, and about 0.1-0.5% by weight of lanolin.

16. A lubricating composition adapted to form a water-in-oil emulsion in the presence of water, with the water in the discontinuous phase, comprising the following ingredients in the listed proportions by weight based on the composition:

|                                                                                        | Per cent     |
|----------------------------------------------------------------------------------------|--------------|
| Mineral lubricating oil                                                                | 94.2 - 99.75 |
| 1-hydroxyalkyl 2-C <sub>10</sub> -C <sub>30</sub> alkenyl glyoxalidine                 | 0.05 - 0.4   |
| Alkylolamine C <sub>16</sub> -C <sub>30</sub> saturated fatty acid ester               | 0.05 - 0.4   |
| Hexahydric alcohol anhydride C <sub>10</sub> -C <sub>30</sub> fatty acid partial ester | 0.1 - 1.0    |
| Linear iso-olefinic polymer having molecular weight over 5000                          | 0.05 - 0.5   |

17. A lubricating composition according to claim 16, wherein the composition also contains about 0.1-0.5% by weight of lanolin, and about 0.3-3.0% by weight of a non-corrosive sulfurized fatty oil extreme pressure agent.

18. A lubricating composition adapted for the lubrication of marine reciprocating steam engines, comprising the following ingredients in the listed proportions by weight based on the composition:

|                                                                | Per cent     |
|----------------------------------------------------------------|--------------|
| Mineral lubricating oil                                        | 94.2 - 99.75 |
| 1-hydroxyethyl 2-heptadecenyl glyoxalidine                     | 0.05 - 0.4   |
| Triethanolamine stearate                                       | 0.05 - 0.4   |
| Sorbitan mono-oleate                                           | 0.1 - 1.0    |
| Linear isobutylene polymer having molecular weight over 10,000 | 0.05 - 0.5   |

19. A lubricating composition according to claim 18, said composition also containing about 0.1-0.5% by weight of lanolin, and about 0.3-3.0% by weight of sulfurized lard oil having about 6-10% of combined sulfur.

20. A lubricating composition adapted for use as a marine engine oil consisting essentially of the following ingredients in the listed percentages by weight based on the composition:

|    |                                                           |      |
|----|-----------------------------------------------------------|------|
| 10 | Mineral lubricating oil                                   | 98.0 |
|    | 1 - hydroxyethyl 2 - heptadecenyl glyoxalidine            | 0.2  |
|    | Sorbitan mono-oleate                                      | 0.2  |
| 15 | Lanolin                                                   | 0.2  |
|    | Triethanolamine stearate                                  | 0.2  |
|    | Isobutylene polymer having molecular weight over 10,000   | 0.2  |
| 20 | Sulfurized lard oil having about 6-10% of combined sulfur | 1.0  |

21. A lubricating composition according to claim 4 also containing about 0.05-0.5% by weight based on the composition of a linear iso-olefinic polymer having a molecular weight in excess of 2,000.

22. A lubricating composition according to claim 21 also containing 0.3-3.0% by weight based on the composition of a non-corrosive sulfurized fatty oil extreme pressure agent which is compatible with said other additives and does not detract from the emulsification properties thereof.

23. A marine engine oil adapted to form a water-in-oil emulsion in the presence of water, with the water in the discontinuous phase, comprising a mineral lubricating oil as the predominant constituent amounting to at least 90% by weight of the composition, about 0.05-0.4% by weight based on the composition of 1-hydroxyethyl 2-heptadecenyl glyoxalidine, about 0.1-1.0% by weight of sorbitan mono-oleate, and about 0.05-0.5% by weight of a linear isobutylene polymer having a molecular weight in excess of 10,000.

45 24. A marine engine oil according to claim 23, also containing about 0.3-3.0% by weight based on the composition of sulfurized lard oil containing about 5-15% of combined sulfur, and about 0.1-0.5% by weight of lanolin.

ROY F. NELSON.  
ALTON J. DEUTSER.  
MELVIN R. HEFTY.

#### REFERENCES CITED

55 The following references are of record in the file of this patent:

#### UNITED STATES PATENTS

| Number    | Name           | Date           |
|-----------|----------------|----------------|
| 1,516,879 | Bezzemberger   | Nov. 25, 1924  |
| 2,193,771 | Puryear        | Mar. 12, 1940  |
| 2,214,152 | Wilkes         | Sept. 10, 1940 |
| 2,268,273 | Wilkes et al.  | Dec. 30, 1941  |
| 2,387,157 | Koppenhoefer   | Oct. 16, 1945  |
| 2,402,373 | Cordero        | June 18, 1946  |
| 2,422,075 | Bray           | June 10, 1947  |
| 2,431,008 | Wright         | Nov. 18, 1947  |
| 2,470,405 | Leland         | May 17, 1949   |
| 2,493,483 | Francis et al. | Jan. 3, 1950   |